

## UNITED STATES PATENT OFFICE

2,078,498

## DENTIFRICE

Emil Klarmann, Bloomfield, and Louis W. Gates,  
Verona, N. J., assignors to Lehn & Fink Products Corporation, Bloomfield, N. J., a corporation of Delaware

No Drawing. Application January 10, 1936,  
Serial No. 58,536

5 Claims. (Cl. 167—93)

The present invention relates to dentifrices and more particularly to dentifrices containing a novel ingredient having a high polishing and cleansing effect and without deleterious abrasive or scratching 5 action on the tooth surfaces.

We have found that the relatively water-insoluble magnesium phosphates having water of crystallization, when finely divided, are especially suitable for use as a dentifrice either alone or in 10 combination with any of the desired and conventional ingredients of a dentifrice. These compounds have a high degree of polishing and cleansing action and are at the same time substantially devoid of abrasive or scratching or 15 other deleterious effects on the enamel or cementum of the teeth.

As stated above, the compounds employed in accordance with our invention are the relatively water-insoluble hydrated magnesium phosphates 20 reduced to a fine particle form as for example the precipitated hydrated tri-magnesium phosphates such as magnesium orthophosphate tetrahydrate  $Mg_3(PO_4)_2 \cdot 4H_2O$ , the magnesium orthophosphate pentahydrate  $Mg_3(PO_4)_2 \cdot 5H_2O$ , and magnesium 25 orthophosphate octahydrate  $Mg_3(PO_4)_2 \cdot 8H_2O$ . While the hydrated tri-magnesium phosphates are preferred, our invention is not to be construed as limited thereto as other water-insoluble hydrated, non-acid magnesium phosphates may 30 be employed as, for example, the hexahydrated magnesium-ammonium phosphate

$(MgNH_4PO_4)_6 \cdot 6H_2O$ .

The compounds embodying our invention, when 35 used as dentifrices per se or in combination with other normal constituents in paste or powder form, are capable of removing the objectionable deposits from and polish the teeth without abrading or scratching the surfaces thereof; and restore and maintain the natural lustre of the teeth. The dentifrice embodying our invention 40 has no deleterious effect on the enamel or cementum of the teeth. These compounds are substantially colorless and tasteless and as stated above are employed in a fine particle form so that all possibility of scratching or abrading the enamel or cementum of the teeth is eliminated.

The following example is illustrative of a typical 45 tooth paste formula containing an insoluble hy-

drated magnesium phosphate as the polishing ingredient:

|                            | Per cent |
|----------------------------|----------|
| $Mg_3(PO_4)_2 \cdot 4H_2O$ | 25       |
| Soap (anhydrous)           | 2        |
| Magnesium hydroxide        | 4        |
| Sugar                      | 13       |
| Glycerine                  | 25       |
| Flavor                     | 1        |
| Water                      | 30 10    |

The following example is illustrative of a typical tooth powder formula:

|                            | Per cent |
|----------------------------|----------|
| $Mg_3(PO_4)_2 \cdot 8H_2O$ | 82       |
| Soap (anhydrous)           | 14       |
| Magnesium hydrate          | 1        |
| Flavor                     | 3        |

It is, of course, to be understood that our invention is not limited to the above compositions 20 as the insoluble hydrated magnesium compound may be used as a dentifrice per se or combined in any desired proportions with other desirable dentifrice ingredients, such as massing agents, diluents, flavoring agents, detergents, emollients 25 and the like.

We claim:

1. A dentifrice containing a substantially water-insoluble hydrated tri-magnesium phosphate in finely divided form so as to act as a 30 polishing and cleansing agent.
2. A substantially non-abrasive dentifrice containing tri-magnesium orthophosphate tetrahydrate in fine particle form.
3. A substantially non-abrasive dentifrice containing tri-magnesium orthophosphate octahydrate in fine particle form.
4. A substantially non-abrasive dentifrice containing hexahydrated magnesium ammonium phosphate in fine particle form.
5. A substantially non-abrasive dentifrice composition containing a substantially water-insoluble hydrated phosphate selected from the class consisting of substantially water-insoluble hydrated tri-magnesium phosphates and hexahydrated magnesium ammonium phosphate in finely divided form so as to act as a polishing and 45 cleansing agent.

EMIL KLARMANN.  
LOUIS W. GATES. 50